

## UNITED STATES PATENT OFFICE

GEORGE A. RICHTER, MILTON O. SCHUR, AND ROYAL H. RASCH, OF BERLIN, NEW HAMPSHIRE, ASSIGNEES TO BROWN COMPANY, OF BERLIN, NEW HAMPSHIRE, A CORPORATION OF MAINE

PROCESS OF CONDITIONING CELLULOUS MATERIAL FOR PREPARATION OF CELLULOSE DERIVATIVES AND PRODUCT OF SAME

No Drawing. Application filed October 9, 1926. Serial No. 140,674.

This invention relates to the preparation of cellulose derivatives, and more especially cellulose esters such as the nitrocelluloses, and has for its object to provide a process of conditioning cellulosic material to render it more economical and satisfactory particularly for the preparation of the lower nitrocelluloses, such as those customarily employed in the manufacture of films, lacquers, artificial silk, and kindred products.

While the process hereinafter described may be practised on various cellulose fibers such as cotton fiber, sulphite fiber, and the like, it may be practised with especial advantage on chemical wood fiber containing a high percentage of alpha or resistant cellulose and which for convenience of designation will hereinafter be termed "alpha fiber."

Such fiber may be produced as described in application for patent, Serial No. 75,522, filed December 1, 1925, by George A. Richter and Milton O. Schur, by treating a raw or unbleached pulp—a usual commercial, unbleached sulphite pulp containing 85% to 88% alpha cellulose, for example—with a solution of caustic soda or equivalent alkaline compound, under the proper concentration, temperature and time conditions. During the treatment, an appreciable portion of the non-alpha cellulose constituent of the pulp is dissolved and removed, resulting in a purified or refined fiber which contains upward of 93% alpha cellulose, and which requires only a relatively small amount of bleach for conversion into a fiber of high whiteness and usable as a new rag or cotton fiber substitute, not only in the preparation of cellulose derivatives of high purity and commercial value, but also in the manufacture of bond, ledger and writing papers of the finest quality.

In certain cases, the alkaline treatment may be supplemented by other treating steps. Thus, it may be desirable, especially when the raw pulp contains a percentage of non-alpha cellulose constituent higher than usual, to pretreat the pulp with an oxidizing solution, e. g., a chlorine solution, to remove a portion of such constituent or facilitate subsequent removal with the alkaline treating solution. Or if an alpha fiber of very high

cellulose content, say, 95% to 98%, is desired, the alkaline treatment may be followed by a second alkaline treatment, as described in application for patent, Serial No. 75,888, filed December 16, 1925, by George A. Richter. 55 By a double alkaline treatment, the quantity of bleach necessary to produce a fiber of high whiteness is further reduced. The bleached, refined fiber serves as an excellent raw material for the preparation of cellulose derivatives. 60

We have discovered that if cellulose fiber, and more particularly an alpha fiber such as hereinbefore described, is conditioned for nitration by suitable treatment, the nitrating characteristics of such fiber are markedly improved. The treatment of the fiber may be carried out by various procedures, but each procedure aims to modify the absorptivity of the fiber. 70

Our theory is that when fiber is highly absorptive, it is attacked readily by the sulphuric acid present in the mixed nitrating acid, partly dissolving or forming unstable esters therewith, which are hydrolyzed and dissolved during subsequent washing of the product, resulting in a low yield and high acid retention. This condition, it is believed, is true to a pronounced degree in the case of alpha fiber, such fiber being more absorptive 75 and spongy as a result of the extraction of appreciable quantities of impurities from the fiber. We have found that, if alpha fiber is rendered less absorptive as by filling the fiber cells and coating the fiber with suitable cellulose coating material, such as cellulose hydrate, regenerated cellulose, or cellulose derivatives, the reacting fiber surface is diminished, the initial attack by the sulphuric acid is retarded, and the nitric acid is allowed to 80 penetrate into the fibers in the proper concentration to form stable nitrates. Such filling materials are nitrated along with the alpha fiber, so that the purity of the product is substantially unaffected thereby. 85

Fiber in a state similar to cotton may possess certain advantages in the preparation of the higher nitrocelluloses (gun cotton, for example), and in point of fact we have found that in the manufacture of gun cotton, uncon- 95 100

ditioned alpha fiber yields very nearly as good results as conditioned alpha fiber, and both conditioned and unconditioned alpha fiber yield nearly the same results as those obtained with the use of high grade cotton linters or cotton; but, for the preparation of the lower nitrocelluloses, conditioned alpha fiber is far superior to unconditioned alpha fiber.

10 While carrying on extensive experimentation with pulps of various types for the production of nitrocelluloses, we have found that when pulp, and more particularly an "alpha" pulp (i. e. a pulp of high alpha cellulose content), is made up into thin sheets or tissue prior to nitration but after being rendered less absorptive by a substantial beating or hydrating operation, the yield upon nitration, and more specifically nitration resulting in the lower nitrocelluloses, increases materially and the coefficient of acid retention by the nitrated cellulose or pulp materially decreases. Furthermore, when the nitrated product is dissolved in a suitable nitrocellulose solvent (for example, in acetone or in amyl acetate), a smooth, homogeneous solution results, from which a better and stronger film may be made than from a solution prepared from nitrocellulose in the preparation of which unbeaten or slightly beaten pulp was utilized as the raw material. While these desirable effects are produced with other pulps, such, for example, as sulphite pulp, they are much more pronounced if alpha pulp is used.

We are aware of the fact that wood pulps of various types and in various forms have been subjected to nitration, but the results which have been obtained have been variable and more or less indifferent. Thus wood pulp has been commonly nitrated in bulk form, in an unbeaten, shredded condition, or as an absorbent sheet. In certain other instances, cotton or rag stock has been prepared in the form of tissue, especially when certain better grades of nitrocellulose products were to be manufactured. When used in tissue form, it has been known that a greater speed in penetration of the fibers by the acid, and consequently greater facility of nitration, is to be had, and in addition the nitrated product dissolves more readily in the nitrocellulose solvents. In the case of cotton or rag pulp, the benefits to be gained by beating or hydrating the fiber prior to nitration are comparatively slight; with unrefined wood pulp, moderate; but in the case of alpha pulp the advantages are very important. In the preparation of nitrating tissue from wood pulp, the moderate advantages of hydration, so far as we are aware, have not been heretofore recognized; and since the alpha fiber is a comparatively new product, our discovery of the beneficial results of hydrating the re-

fined pulp is undoubtedly a new contribution to the art.

In accordance with the present invention, therefore, the cellulosic pulp is beaten to a high degree of "slowness" prior to its sheeting into tissue for nitration on paper-forming machinery. In actual practice, the pulp is beaten to a slowness of, say, about nine minutes to twelve minutes, this value approximating that of a beaten stock to be used in the manufacture of high grade bond and ledger papers. The beaten pulp is then formed, without the introduction of size, filler or other materials into the stock, into "waterleaf" tissue sheets, and in this form is especially suitable as a raw material for the preparation of the lower nitrocelluloses. Alpha pulp, in particular, when beaten and formed into water-leaf tissue, shows a material increase in yield of nitrated product and a materially lower coefficient of acid retention\* of the spent nitrating acid by the nitrocellulose product, as the slowness or extent of beating of the stock is increased. For example, the yield and acid retention for thin sheets of unbeaten alpha pulp cut into  $\frac{1}{4}$ -inch squares are, respectively, about 136 and 7.6, as compared with a yield of 150 to 155 and an acid retention of 4.0 when the alpha pulp is beaten to a slowness of about nine minutes. The importance of beating prior to nitration is much more pronounced with alpha pulp than with sulphite fiber. Thus the yield and acid retention for thin sheets of unbeaten sulphite pulp of similar size to the pieces of alpha pulp are, respectively, 145 and 4.5 to 5.5; for sulphite pulp beaten to a slowness of eight minutes, 145 to 150 and 3.5 to 4.0. The more pronounced changes in yield and lessened acid retention produced by the beating of alpha pulp for purposes of nitration may be imputed to the fact that alpha pulp is considerably purer and more absorptive to begin with than sulphite or other commercial pulp ordinarily employed.

The comparative values hereinbefore given were obtained by the use of a nitrating acid suitable for the preparation of the lower nitrates and consisting of:

|                               | Per cent | 115 |
|-------------------------------|----------|-----|
| $\text{HNO}_3$ -----          | 20.5     | 115 |
| $\text{H}_2\text{SO}_4$ ----- | 60.8     |     |
| $\text{H}_2\text{O}$ -----    | 18.7     |     |

(the ratio of acid used to fiber being 50 to 1). The nitration was carried out at 40° C. for thirty minutes.

While more power must be expended in beating alpha pulp to a given slowness than when beating sulphite pulp, the use of alpha pulp as a raw material for the production of

\* The coefficient of acid retention is the percent of the weight of the original nitrating acid retained by the nitrated cellulose when centrifuged under carefully standardized conditions. It is a direct measure of the loss in nitrating acid experienced in usual technical practice when the centrifuged material is drowned in large volumes of water.

nitrocelluloses results in a product of much higher purity.

By the term "alpha pulp" as herein employed is meant a pulp containing at least 93% alpha cellulose, having a copper number below 2.5, and possessing excellent paper-making qualities and certain other very desirable characteristics. Among such characteristics, such pulp should possess the following:

|                                                                                                    | Per cent |
|----------------------------------------------------------------------------------------------------|----------|
| "Soda solubility" (amount of fiber dissolved at boiling temperature in 7.14% NaOH solution), under | 12       |
| Ash content, under                                                                                 | 0.4      |
| 15 Resin content, under                                                                            | 0.4      |

When confetti prepared from pulp possessing the characteristics hereinbefore given, and beaten to a slowness of about nine minutes, 20 is nitrated, the nitration proceeds smoothly, the mixed acids being absorbed readily and uniformly. The resulting nitrocellulose dissolves readily in nitrocellulose solvents such as in acetone and amyl acetate, for example, 25 resulting in solutions of relatively low viscosity and of good color. When the solution is spread over a smooth surface and the solvent allowed to evaporate, a light colored film of good strength is obtained, comparable in 30 respect of clearness, strength and color to films prepared from cotton fiber, and in these respects is superior to films made from sulphite or other pulps of lower purity or alpha cellulose content.

35 In carrying on experimental work connected with our discovery, we have found that a relatively large rate of increase in yield, and large drop in acid retention of the nitrocellulose, occurs at the earlier portion 40 of beating, the rate of such changes decreasing as the amount of beating is increased. The more the pulp is beaten (that is, the slower the pulp), the greater the change in 45 these factors throughout the range experienced with, although for all practical purposes the pulp need not be beaten beyond a slowness of about nine to twelve minutes, the cost of additional beating then overbalancing the desirable effects gained. In order to 50 secure thorough penetration of the beaten pulp by the nitrating acid in a minimum period of time (that is, in a thirty-minute time period allotted for nitration in the instant case), it is essential that the thin 55 sheeted pieces or tissue be light, preferably below 20 in basis weight (480-24×36), or equivalent to a thickness of about .003 inches. When such material is subjected to the conditions hereinbefore stated, the effect of a 60 substantial beating of alpha pulp prior to nitration is very remarkable and advantageous, in that the yield of nitrocellulose product may be increased from about 136% to a 65 yield of 157%, and the acid retention lowered from about 7% to 4%, more or less.

We have also discovered that, if cellulose fiber (and more particularly alpha fiber) is hydrated by mercerization in a solution of caustic soda, the nitrating characteristics of such fiber are markedly improved.

70 For instance, the fiber may be fluffed mechanically to resemble cotton linters, or may be in the form of a thick sheet formed on a cylinder machine from a very dilute suspension of pulp, and dried on the mould, either with or without squeezing. The alpha fiber in fluffed condition may, for example, be steeped in a caustic soda solution of 17.5%, or greater, strength, at 20° C., for 30 minutes, followed successively by a 75 washing with cold water, a souring with 20% acetic acid solution, and a final washing with hot water. The product may then be dried and nitrated into the lower nitrocelluloses with mixed acids of the desired strength. 80

When fiber which had been mercerized by the treatment set forth in the example was nitrated, an increase in yield from 136 to 141, a lowering of the acid retention from 6.7 to 5.5, a decrease in the viscosity of the solution 90 of nitrocellulose product and a marked improvement in the color of the solution were noted.

The mercerizing treatment may, of course, be varied. Thus, the time of mercerization 95 may be five minutes or less, and the washing after mercerization may be done with hot water. The results attained upon nitration, in any event, however, indicate an increase in yield, a material lowering of the acid retention, and a marked improvement in color and other characteristics of the nitrated product. Thus, mercerization of a mechanically fluffed sheet of alpha fiber, prepared on a cylinder machine, for three to five minutes in a solution of caustic soda of 18% strength, followed by hot washing, acid souring and cold washing, produce upon nitration an increase 100 in yield from 125 to 142, a decrease in acid retention from 8.4 to 5.5, and a marked improvement in the color of the product. 110

Mercerization effects a change in the character of the fiber which upon nitration asserts itself in a lower acid retention and a higher 115 yield of nitrocellulose product. The product is of high purity and consequently produces a smooth, homogeneous and clear solution in a nitrocellulose solvent, from which better and stronger films and other products may be prepared than from solutions formed 120 from unmercerized fiber. One factor contributing to these results doubtless is that during mercerization a further removal of non-alpha cellulose constituents in the alpha fiber is effected, and hence there results a 125 purer nitrocellulose, from which better lacquers, films or plastics may be produced.

The superior product, as well as the higher yield and lower acid retention may also be imputed to the change in physical character- 130

istics which mercerization effects on the fiber. Our theory is that both beating and mercerization of the fiber which produce hydrocellulose or an incipient gelatinization of the fiber, yield a denser or less absorptive fiber which resists the initial attack of the mixed nitrating acid. Mercerization appears to effect results similar to beating, and, if desired, may be combined with a beating of the fiber, so that advantages incident to both may be realized.

The best results are obtained when the alpha fiber is both beaten and mercerized. Mercerized alpha fiber yields nitrocellulose from which films and other products may be prepared having properties comparable to those obtainable with good grade cotton linters or with a moderately high grade rag sheet.

Our mercerized fiber conditioned for nitration has, among others, the following characteristics:

|                                                                                                |        |
|------------------------------------------------------------------------------------------------|--------|
| Alpha cellulose content, over                                                                  | 94.5 % |
| Soda solubility (amount of fiber dissolved at boiling temperature in 7.14 NaOH solution) under | 10.0 % |
| Copper number, under                                                                           | 2.2    |
| Ash, under                                                                                     | 0.2 %  |
| Resins, under                                                                                  | 0.25%  |
| Pentosans, under                                                                               | 2.0 %  |

We are, of course, aware of the fact that mercerization of cellulose material is in itself broadly old, but, so far as we are aware, the beneficial results obtainable by combining the mercerization of wood fiber, and more especially a high alpha cellulose fiber, with nitration, have not heretofore been recognized.

The advantages of our process may be extended to the production of other cellulose esters, such, for example, as cellulose acetate, for the mercerization of cellulose followed by a hot water treatment as hereinbefore described will improve materially the smoothness of acetylation and the quality of cellulose acetate obtained, particularly with regard to the elimination of undesirable color.

We have further discovered that if cellulose fiber, and more particularly an alpha fiber such as hereinbefore described, is rendered less absorptive for nitration by treatment with suitable filling materials such as nitrocellulose or regenerated cellulose, prior to nitration, the nitrating characteristics of such fiber are markedly improved. The fiber may be treated while in either bulk or sheet form, and then nitrated in either form, but, inasmuch as nitration proceeds most favorably when the fiber is in the form of thin sheet or nitrating tissue, nitration is preferably performed on the fiber when in this condition.

The filling of the fiber may be accomplished while it is in sheet form by various methods, but each aims to accomplish the filling of the fiber cells and the coating of the fiber with nitrocellulose or regenerated cellulose. Thus, a thin waterleaf sheet made from alpha fiber may be treated by immersion in a relatively dilute solution of nitrocellulose in acetone or other solvent of, say, 1/5% to 1/4% concentration. The treatment may be carried out until the sheet has absorbed or retained the desired amount of nitrocellulose. The nitrocellulose filled sheet may then be dried, cut up into small squares or confetti, suitable for nitration.

Or cellulose may be regenerated in situ on the fiber and in the fiber cells by precipitation from a solution of suitable cellulose derivative. For example, a waterleaf sheet of alpha fiber may be passed through a solution of viscose of, say, 1% cellulose concentration. The sheet may be completely dried or else partially dried, and then passed through a suitable setting bath, e. g., a solution of acetic acid or sodium bisulphate and sulphuric acid, thereby effecting a precipitation of regenerated cellulose in situ on the fiber and in the fiber cells. The sheet may then be washed substantially free of acid, steeped if desired in a sulphide-removing bath, e. g., a sulphite solution, again washed, dried, and cut up into squares or confetti suitable for nitration.

The treatment of the fiber may be carried out while such fiber is in bulk or shredded condition. Thus, finely shredded alpha fiber may be uniformly treated with a solution of cellulose nitrate in acetone of, say, 1/4% concentration. The fiber may then be nitrated in this condition.

Or the finely shredded fiber may be treated with a viscose solution of, say, 1% cellulose concentration. The excess solution may be expressed from the mass by centrifuging, whereupon the mass may be completely dried or else partially dried, then treated with a suitable setting solution. The fiber may then be washed substantially free of acid, steeped if desired in a sulphide-removing bath, again washed, dried, and finally nitrated.

Or the finely shredded fiber may be treated with a solution of nitrocellulose as in an alcohol-ether mixture, then denitrated by treatment with a strong solution of ammonium polysulphide for, say, one hour, at 80° F., washed, neutralized, again washed, thickened, dried, and finally nitrated. Sheeted fiber may be similarly treated. Cellulose may also be regenerated on sheeted or bulk fiber from a cuprammonium-cellulose solution.

Another procedure of treating fiber may be carried out similarly to the usual beater sizing process. In this case, a cellulose deriva-

tive, e. g., viscose, may be added to the alpha fiber in the beater engine, preferably after it has been beaten, and may then be uniformly disseminated throughout the fiber by the operation of the engine. Regenerated cellulose may then be precipitated on the fiber and fiber cell wall, by the addition of a suitable precipitating agent, e. g., an acid mixture or acid salt, whereupon the fiber may be washed prior to sheeting. The fiber may then be sheeted into waterleaf paper suitable for nitration.

Filled alpha fiber, such as hereinbefore described, when nitrated results in a high yield of nitrocellulose and is accompanied by lower acid retention than similar unfilled fiber. The filling treatment may be controlled to incorporate, say, 5% to 10% filling material into the fiber, but even 1% yields noteworthy improvement in nitrating characteristics. The nitrocellulose produced from the conditioned fiber is of high purity, and accordingly produces smooth homogeneous and clear solutions in nitrocellulose solvents, from which better and stronger films and other products may be made than from solutions formed from nitrocellulose produced from similar unfilled fiber.

Filling the fiber with gelatinized cellulose or cellulose esters is also beneficial in the manufacture of esters other than the nitrate, leading to a higher yield of more uniform product.

Of course, if desired, a certain proportion of cotton linters, cotton, or rag pulp may be mixed with the alpha fiber. Thus, cotton fiber and alpha fiber may be mixed and treated with suitable filling materials prior to nitration, or may be mercerized prior to nitration, or first beaten together, then mercerized, and finally nitrated.

The present invention makes possible the use of a high alpha cellulose fiber, which may be manufactured at a figure materially lower than that at which cotton linters or cotton are available, for the production of high grade nitrocellulose products.

Having thus explained the nature of this invention, it is evident that various changes might be resorted to without departing from its spirit or scope as defined by the appended claims.

We claim:

1. A process of producing a cellulose derivative from a high alpha cellulose wood fiber, which comprises rendering the fiber less absorptive with a cellulose coating material and then converting the fiber into the derivative.

2. A process of producing nitrocellulose from a high alpha cellulose wood fiber, which comprises rendering the fiber less absorptive with a cellulose coating material, and then nitrating the fiber.

3. A process of producing a cellulose derivative from a high alpha cellulose wood

fiber, which comprises filling the fiber cells and coating the fiber with gelatinized cellulose, and then converting the fiber into the derivative.

4. A process of producing nitrocellulose from a high alpha cellulose wood fiber, which comprises filling the fiber cells and coating the fiber with gelatinized cellulose, and then nitrating the fiber. 70

5. That step in the production of cellulose derivatives from wood pulp, which comprises beating such pulp to about the slowness of pulp used in bond paper manufacture prior to conversion into its derivatives. 75

6. That step in the production of cellulose derivatives from high alpha cellulose wood pulp, which comprises beating such pulp to about the slowness of pulp used in bond paper manufacture prior to its conversion into its derivatives. 80

7. A process which comprises beating wood pulp to about the slowness of pulp used in bond paper manufacture and then nitrating such pulp. 85

8. A process which comprises beating a high alpha cellulose pulp to about the slowness of pulp used in bond paper manufacture, and then nitrating such pulp. 90

9. A process which comprises beating wood pulp to a slowness of about nine minutes and then converting said pulp to a cellulose derivative. 95

10. A process of producing cellulosic material especially adapted for conversion into cellulose derivatives, which comprises beating a high alpha cellulose wood pulp to about the slowness of pulp used in bond paper manufacture prior to its conversion into a cellulose derivative. 100

11. A process which comprises beating wood pulp to about the slowness of pulp used in bond paper manufacture and then forming such pulp into thin sheets prior to conversion into cellulose derivatives. 105

12. A process which comprises beating wood pulp to about the slowness of pulp used in bond paper manufacture, forming such pulp into tissue suitable for nitration, and then nitrating such tissue. 110

13. A process which comprises beating wood pulp to about the slowness of pulp used in bond paper manufacture, forming such pulp into tissue suitable for nitration, cutting such tissue into small pieces, and then nitrating such pieces. 115

14. A process which comprises beating a high alpha cellulose wood pulp to a slowness of about nine minutes, and then forming such pulp into thin sheets of tissue suitable for nitration. 120

15. A process which comprises beating a high alpha cellulose wood pulp to a slowness of about nine minutes, forming such pulp into tissue suitable for nitration, and cutting such pulp into small pieces. 125

16. A process which comprises beating a high alpha cellulose wood pulp to about the slowness of pulp used in bond paper manufacture, forming such pulp into nitration tissue, nitrating such tissue, dissolving the nitrocellulose product in a nitrocellulose solvent, and forming a nitrocellulose product from said solution.
17. A waterleaf tissue especially suitable for nitration, comprising wood pulp beaten to a slowness of about nine minutes.
18. Material especially suitable for nitration, comprising unfilled and unsized high alpha cellulose wood fiber beaten to about the slowness of pulp used in bond paper manufacture.
19. A waterleaf tissue especially suitable for nitration, comprising high alpha cellulose wood fiber beaten to about the slowness of pulp used in bond paper manufacture.
20. Material especially suitable for nitration, comprising unfilled and unsized high alpha cellulose wood fiber beaten to a slowness of about nine minutes.
21. A waterleaf tissue especially suitable for nitration, comprising high alpha cellulose wood fiber beaten to a slowness of about nine minutes.
22. An unfilled, unsized paper especially suitable for nitration, comprising wood pulp beaten to about the slowness of pulp used in bond paper manufacture.
23. An unfilled, unsized paper especially suitable for nitration, comprising high alpha cellulose wood pulp beaten to about the slowness of pulp used in bond paper manufacture.
24. A waterleaf tissue especially suitable for conversion into nitrocellulose, comprising a high alpha cellulose wood fiber beaten to about the slowness of pulp used in bond paper manufacture and possessing the following characteristics, to wit:
- |                                                |      |
|------------------------------------------------|------|
| Alpha cellulose content, over                  | 93 % |
| 45 "Soda solubility" (in 7.14% NaOH),<br>under | 12 % |
| Copper number, under                           | 2.5  |
| Ash, under                                     | 0.4% |
| Resins, under                                  | 0.4% |
25. A waterleaf especially suitable for conversion into cellulose derivatives, comprising a high alpha cellulose wood fiber beaten to a slowness of about nine minutes and possessing the following characteristics, to wit:
- |                                                |      |
|------------------------------------------------|------|
| Alpha cellulose content, over                  | 93 % |
| 55 "Soda solubility" (in 7.14% NaOH),<br>under | 12 % |
| Copper number, under                           | 2.5  |
| Ash, under                                     | 0.4% |
| 60 Resins, under                               | 0.4% |
26. A nitrocellulose product, the cellulosic base of which comprises a high alpha cellulose wood pulp beaten to about the slowness of pulp used in bond paper manufacture.
27. A process which comprises coating the fibers of wood pulp with a cellulosic material and then converting the pulp into cellulose derivatives.
28. A process which comprises coating the fibers of wood pulp with a cellulosic material and then nitrating the pulp.
- In testimony whereof we have affixed our signatures.
- GEORGE A. RICHTER.  
MILTON O. SCHUR.  
ROYAL H. RASCH.